

Dec. 4, 1951

K. M. BARTLETT

2,577,644

## APPARATUS FOR ANODICALLY TREATING INTERNAL SURFACES

Original Filed April 9, 1943



Inventor  
Kenneth M. Bartlett.

By Charles Wells ATHS.

## UNITED STATES PATENT OFFICE

2,577,644

APPARATUS FOR ANODICALLY TREATING  
INTERNAL SURFACESKenneth M. Bartlett, Cleveland, Ohio, assignor to  
Thompson Products, Inc., a corporation of OhioOriginal application April 9, 1943, Serial No.  
482,379. Divided and this application May 7,  
1949, Serial No. 93,517

1 Claim. (Cl. 204—222)

1

This is a division of application Serial No. 482,379 filed April 9, 1943, now abandoned.

This invention relates to an apparatus for anodically treating internal surfaces, and more particularly to the anodic descaling of internal surfaces of a hollow metal valve.

In the manufacture of hollow metal valves, either by forging or casting methods, it has generally been found necessary to clean the internal surfaces of the head cavity of the valve in order to free such surfaces from scale resulting from the forging and heat treatment and to provide surfaces having a high rate of heat transfer between the walls of the head of the valve and the coolant with which the valve may be partially filled. Various methods of cleaning the internal surfaces of the head cavity of hollow valves have been devised, such as sand blasting, or other mechanical methods, but these have proved rather unsatisfactory.

I have now found that it is possible by the use of an anodic electrolytic method to descale the internal surfaces of hollow metal valves, and particularly the internal surfaces of the head cavity. In accordance with the present invention, a collapsible cathode is inserted into the hollow metal valve to provide conducting means extending adjacent to and in general conformity with the interior walls of the head cavity. Preferably, a hollow or tubular member is employed for supporting the collapsible cathode within the head cavity, in order that the electrolyte used may be introduced into the interior of the valve through such hollow or tubular member. The valve is then made the anode and an electrical current passed through the electrolyte from the anode to the cathode of sufficient current density and for a sufficient length of time to effect a complete descaling of the walls of the head cavity of the valve. There is thus provided a simple yet effective method for descaling the interior wall surfaces of a hollow metal valve, without the necessity of employing mechanical cleaning or descaling means.

It is a further important object of this invention to provide apparatus for use in the anodic descaling of internal surfaces of a hollow metal object, such as a hollow metal valve, which apparatus includes a tubular member for the introduction of the electrolyte into the interior of the valve and a collapsible cathode carried by the end of said tubular member and adapted, when extended, to lie adjacent to the walls of the valve head and in general conformity therewith.

2

Other and further important objects of this invention will be apparent from the disclosures in the specification and the accompanying drawings.

5 On the drawings:

Figure 1 is an elevational view, partly broken away and in section, of a form of apparatus adapted for carrying out the method of my invention;

10 Figure 2 is an enlarged, fragmentary, sectional view of the valve itself and the attachments therefor, with parts broken away and in section and with parts in elevation; and

15 Figure 3 is an enlarged, fragmentary detail view of the collapsible cathode used in the apparatus of my invention.

The reference numeral 10 indicates generally a supporting stand, such as a ring stand, having a base 11 and an upright rod 12, on which 20 are adjustably mounted a plurality of clamping members. One of said clamping members, indicated by the reference numeral 13, is adapted to support the hollow metal valve 14 in substantially vertical position with the head end 25 15 at the bottom and the open stem end 16 at the top. Said clamping member 13 is adjustable along the rod 12 by means of a thumbscrew 17. The supporting end of the clamping member 13 is an integral ring 18 having an annular lining 19 of rubber or other insulating material. The stem portion 16 of said valve 14 is adapted to be inserted into the opening provided by said lining 19 and to be frictionally held therein.

30 Another clamping member 20 serves to support a reservoir 21 for containing an electrolyte 22. Said reservoir 21 is suitably provided with a stop cock 23 for controlling the flow of electrolyte through a flexible hose 24 into a tubular member 25 that extends into said hollow valve 14. The tubular member 25, which may be formed of stainless steel, copper or other electrical conductive materials, is supported above the valve 14 by means of a clamping member 26, from which it

40 is insulated by an insulating sleeve 27. An apertured spacer 28, positioned in the stem end 16 of said valve 14, permits the tubular member 25 to be inserted therethrough and serves to center and space said tubular member from the walls of the valve. A similar, apertured spacer 29 is adapted to be positioned within said hollow valve 14 near the end of the stem cavity 30 thereof. Said spacers 28 and 29 are provided with fluid flow passages 31 and 32, respectively, and also with apertures 50 33 and 34 for a purpose that will later appear.

## 3

The tubular member 25 is provided with a stop-off coating 35 for the portion of its length that extends within said hollow valve 14. The purpose of this stop-off coating is to prevent contact between the external surface of said tubular member 25 and the electrolyte with which the hollow valve 14 is filled during the anodic descaling process. In the particular process about to be described, wherein the walls of the head cavity only are to be anodically treated, it would be undesirable to have the external portions of the tubular member 25 in electrical contact with the electrolyte, since that would mean a considerable loss in current between the walls of the stem portion of the valve and the tubular member. 10 Where, however, the tubular member 25, or its equivalent, is to be used as a cathode, as in my copending application Serial No. 482,378, filed April 9, 1943, now Patent No. 2,475,586, the stop-off coating would be omitted, and in that case 20 the internal walls of the stem cavity 30 could be anodically treated in accordance with the electro-polishing method of my copending application.

The lower end of the tubular member 25 is provided with a pin 36 extending laterally therefrom, to which is hingedly attached a metal strip link 37, which may suitably be a strip of stainless steel about three-sixteenths of an inch in width. A similar strip of stainless steel 38 is hingedly connected, as at 39, to the free end of said strip 37. The hinge 39 may be formed in any suitable way, as by providing a pin 40 about which portions of the strips 37 and 38 are bent for relative pivotal movement. A stainless steel wire 41 is connected to the free end of the strip link 38, as at 42, by a similar hinge connection. Said wire 41 extends from the hinge connection 42 through the openings 34 and 33 respectively, in the spaces 29 and 28, in order to provide an extension portion 43 that may be manually manipulated to collapse or extend the links 37 and 38. By pulling up on the wire 43, the links 37 and 38 are collapsed into their more or less straight-line position, as illustrated in Figure 3, whereas when the wire 43 is depressed, the link 38 is extended laterally to conform in general with the contour of the end wall 44 of the head cavity 45 of the valve, and the link 37 is brought into an inclined position adjacent to and, in general, conforming with the taper of the neck wall 46 of said valve. The links 37 and 38, as will later be described in more detail, thus form the active cathode electrode in the anodic descaling of the walls of the head cavity 45.

In carrying out the anodic descaling of the internal walls of the valve cavity 45, the valve 14 and the tubular member 25 are made a part of an electrical circuit, including lead wires 47 and 48, connected, respectively, to the positive and negative terminals of a source of direct electric current. A switch 49 is positioned in the line 47, which is connected through an ammeter 50 and a rheostat 51 to the valve 14 by means of a clamping band 52. The line 48 is connected to a bare portion of the tubular member 25 by means of a clamping member 53. A voltmeter 54 is connected across the lines 47 and 48 by means of a line 55.

In operation, the reservoir 21 is provided with an aqueous electrolyte, preferably heated to a temperature of between about 50° and 150° F. The electrolyte that I prefer to use is an aqueous solution of orthophosphoric acid, containing about 75% of orthophosphoric acid by weight of the solution. Other aqueous electrolytes may,

however, be used satisfactorily, such as sulphuric acid, or mixtures of sulphuric and phosphoric acids. The choice of the electrolyte will depend, in part, upon the metal or alloy of which the valve 14 is formed.

Suitable metals and their alloys that might be used in the manufacture of hollow metal valves, such as the valve 14, include: nickel, chromium, and iron alloys such as Nichrome steel; nickel, molybdenum and iron alloys such as Hastelloy steel; non-ferrous nickel-chromium alloys such as Brightray; and cobalt, chromium and tungsten alloys, such as Stellite. I prefer to use orthophosphoric acid in the descaling of valves made of any of the foregoing metals or alloys.

At the start of the operation, the stop cock 23 is opened to permit the electrolyte 22 to pass through the flexible hose 24 into the tubular member 25, and thence into the interior of the valve 14. After the interior of the valve 14 has been filled with the electrolyte, the stop cock 23 is adjusted to permit a continuous, slow overflow of the electrolyte through the overflow opening 31 in the top spacer 28. The rate of flow is not particularly important, but I have found that a flow of about 2 cc. of electrolyte per minute is satisfactory. The excess of electrolyte that overflows through the opening 31 runs down over the outside of the valve 14 and drips into a catch basin 56.

As soon as the rate of flow of electrolyte has been adjusted, the circuit including the lines 47 and 48 is energized to pass an electrical current from the valve 14 as the anode, through the electrolyte filling the interior of the valve, to the active cathode consisting of the links 37 and 38. Since the portion of the tubular member 25 is coated with a stop-off lacquer or the like throughout the portion of said tubular member that is immersed in the electrolyte, no electrolytic action takes place at the external surface of said tubular member 25, but is confined to the links 37 and 38 and, to a slight extent, to the wire 41. The tubular member 25 nevertheless forms a conductor for the current back to the lead wire 48 through the clamping connection 53.

The current is applied to the internal circuit including the electrolyte at an applied voltage of around 4 volts, and the amperage is regulated by means of the rheostat 51 to deliver a current of about 5 amperes. During the course of the anodic treatment, which may require around forty-five minutes, the cathode electrode, comprising the strip links 37 and 38 is rotated through about 45° every five minutes. This may be accomplished either by revolving the tubular member 25 together with the spacers 28 and 29 that are frictionally rotatable with said tubular member 25, or, more easily, by rotating the valve 14 within the ring support 18. For this latter purpose, the clamping member 52 may be loosened, if necessary. The purpose of the rotation of the active cathode electrode is to secure uniform descaling of the interior wall of the valve head cavity 45.

At the completion of the descaling operation, the electrical circuit is de-energized, the valve 14 disconnected from the electrical clamping member 52 and removed from the ring support 18. The electrolyte is poured out of the valve 14 and the valve then thoroughly rinsed in hot water until free from electrolyte. After the hot water rinse, the scale will be found to have been completely removed from the valve head interior and the surface will have a bright finish. While

there may be a pitting effect due to the anodic action on the metal of the wall surface, such effect is not objectionable.

As mentioned above, the method of this application is somewhat analogous to that described and claimed in my Patent No. 2,475,586. In the electropolishing of the internal wall of the valve stem, as described in said patent, orthophosphoric acid is also used as the electrolyte and the operating conditions are somewhat similar to those specified herein, except that a slightly lower current density is employed. In electropolishing, as distinguished from descaling, a proper value of current density is required to strike a practical balance between the time required to polish and the time within which pitting of the surface occurs at relatively high density. In the descaling operation, as here described, a relatively high current density is used to keep the operating time within practical limits.

The same apparatus and practically the same conditions as herein described could, therefore, be used for the electropolishing of the internal surfaces of the valve head cavity 45, if that were desired. Practically the only change to be made in order to effect electropolishing would be to lower the current density by decreasing the current to about 2.5 to 3.5 amperes per valve, instead of 5 amperes. With a current of between 2.5 and 3.5 amperes per valve, the current density will run about 0.5 ampere per square inch, so that with 5 amperes per valve, as in the descaling operation, the current density would be about 1 ampere per square inch.

The above described method of descaling the internal wall of the head cavity of a valve eliminates one of the greatest problems in the manufacture of hollow head valves for use with metal coolants, such as sodium. The presence of scale in the interior of the hollow valve is very detrimental, since it contaminates the sodium and also greatly interferes with the cooling of the valve in the operation of an engine. By removing the scale, a surface having a much more efficient rate of heat transfer is obtained. Furthermore, by the anodic descaling treatment of the interior surfaces of the wall of the valve, these surfaces are rendered more corrosion resistant and therefore less liable to attack by the liquid sodium most commonly used in the cooling of hollow valves.

While the method of my invention has been

described in connection with the use of direct current, it is also possible, although not preferred, to use an interrupted or reversing direct current or even an alternating current to effect the cleaning or descaling of the internal surface of the valve head.

It will, of course, be understood that various details of construction may be varied through a wide range without departing from the principles of this invention and it is, therefore, not the purpose to limit the patent granted hereon otherwise than necessitated by the scope of the appended claim.

What I claim is:

- 15 Apparatus for effecting an anodic treatment of the internal surfaces of a hollow metal article having an enlarged head cavity, comprising an electrically conductive tubular member, a pair of spacers in spaced relation along said tubular member, each of said spacers having a fluid flow passage therein and an aperture to slidably receive an actuating wire therethrough, means for introducing a flow of an electrolyte through said tubular member, a collapsible conductive extension secured to one end of said tubular member, an actuating wire having one end secured to said collapsible conductive extension and extending through the apertures in said spacers in parallel spaced relationship to said tubular member for collapsing and extending said collapsible conductive extension, whereby when said apparatus is inserted in a hollow metal article, an electrolyte introduced through said tubular member will flow about said conductive extension and then through the fluid flow passages in said spacers.

KENNETH M. BARTLETT.

#### REFERENCES CITED

- 40 The following references are of record in the file of this patent:

#### UNITED STATES PATENTS

|    | Number    | Name       | Date          |
|----|-----------|------------|---------------|
| 45 | 950,579   | Seitz      | Mar. 1, 1910  |
|    | 2,332,569 | Greenslade | Oct. 26, 1943 |

#### FOREIGN PATENTS

|    | Number    | Country   | Date          |
|----|-----------|-----------|---------------|
| 50 | 15,963/34 | Australia | Jan. 16, 1934 |
|    | 634,410   | Germany   | Aug. 26, 1936 |